

July 7, 1925.

1,544,544

N. M. AUSTIN

METHOD OF MAKING CASTINGS

Filed March 5, 1923

*Fig. 1.*



*Fig. 3.*



*Fig. 2.*



*Fig. 4.*



INVENTOR

Ned M. Austin  
By Byrnes, Abbott & Carmichael

His  
Atty's

Patented July 7, 1925.

1,544,544

# UNITED STATES PATENT OFFICE.

NED M. AUSTIN, OF CANTON, OHIO, ASSIGNOR TO UNITED ENGINEERING AND FOUNDRY COMPANY, OF PITTSBURGH, PENNSYLVANIA, A CORPORATION OF PENNSYLVANIA.

## METHOD OF MAKING CASTINGS.

Application filed March 5, 1923. Serial No. 622,841.

To all whom it may concern:

Be it known that I, NED M. AUSTIN, a citizen of the United States, residing at Canton, in the county of Stark and State of Ohio, have invented a new and useful Improvement in Methods of Making Castings, of which the following is a full, clear, and exact description.

The present invention relates broadly to the art of molding, and more particularly to an improved method of making castings. In making certain types of castings, particularly cast rolls, it has heretofore been the practice, in order to obtain the desired depth of chill, to employ a composition of metal having the property of freezing quickly. The quick freezing, however, does not allow sufficient time for the graphite to separate out enough to give a solid gray interior to the casting. The quick freezing also has a tendency to set up casting strains which, when a casting is broken, show in the form of radial streaks from the surface towards the center.

By the present invention I propose to overcome the above mentioned and other disadvantages of the prior practice, by effecting a change in the chemical and physical interior structure of a casting after the molten metal has been poured into the mold, and preferably after the superficial portion of the molten metal has cooled and solidified to form an outer shell. This change is produced by causing the diffusion into the interior of the molten metal of a different metal or material. The invention is of particular importance in connection with the casting of rolls, it being desirable, for example, to lower the melting point of the metal of which the interior of the casting is composed in order that this portion of the casting will not cool too quickly.

Two slightly different methods for practising my invention are illustrated in the accompanying drawings, in which—

Figures 1 and 2 are similar vertical sectional views of a mold illustrating one method of carrying my invention into effect;

Figure 3 is a view similar to Figures 1 and 2, illustrating a slightly modified method; and

Figure 4 is a sectional view of a roll casting made in accordance with my invention.

Referring to the drawings, A represents an ordinary sand mold, which may have one or more mold cavities, for casting rolls. This mold has the usual pouring basin 1, strainer core 2, and the vertical and horizontal passages 3 and 4, constituting the gate, for introducing the molten material into the mold, and the riser vents 5. While I have shown a mold for casting rolls, it will be understood that my invention is not limited to rolls, but is applicable to castings generally, irrespective of shape or intended use.

In accordance with the method illustrated in Figures 1 and 2, a pipe 6 is introduced into the mold through a riser vent 5 prior to the pouring of the molten metal into the mold. The lower end of the pipe is closed by a wall of the mold, and the pipe is of some material which will not melt when subjected to the heat of the molten metal surrounding the pipe. The molten metal is now poured into the mold and the superficial portion of the metal surrounding the pipe may be allowed to cool and solidify to form an outer shell. Then the pipe 6 is filled with molten material, which may be another metal, for instance, and the pipe gradually withdrawn from the mold to allow the molten material contained within it to diffuse into the molten metal in the interior of the shell, thereby changing the composition of the casting up to the frozen shell.

In Figure 3 I have illustrated a slight modification of the above described method. According to this method, a bar 7 of different chemical analysis is inserted down through a molten mass of metal in a mold, said bar melting and diffusing into the surrounding metal as in the first method.

It will be understood, of course, that in the case of rolls the object is to obtain extreme hardness in the outer portion of the roll for a considerable depth while giving to the interior of the roll great tensile strength. By the introduction of various metals, in the manner above described, and containing varying proportions of silicon, manganese, carbon, chromium, molybdenum, nickel, copper, cobalt, tungsten, titanium, aluminum and the like, I am enabled to change the internal structure of a roll casting so as to greatly increase the strength of the roll, and I am at the same time enabled to chill to

the desired depth. In fact, the present invention enables chilling to greater depths than formerly without weakening the roll.

In Figure 4 I have illustrated a roll casting made in accordance with either of the methods above described.

I claim:

1. The method of making a casting, which comprises causing the diffusion into the 10 interior of a mass of molten metal in a mold of material adapted to change the internal structure of the casting, substantially as described.

2. The method of making a casting, 15 which comprises filling a mold with molten metal, allowing the superficial portion of the metal to cool and solidify to form a shell, and then causing the diffusion into the interior of the molten metal of material 20 adapted to change the internal structure of the casting, substantially as described.

3. The method of making a casting, which comprises providing a mass of molten metal in a mold with a core composed of material 25 adapted to diffuse into said molten metal and change the internal structure of the casting, substantially as described.

4. The method of making a casting, which comprises causing the diffusion into the 30 interior of a mass of molten metal in a mold, of material adapted to lower the melting point of the interior portion of the casting, substantially as described.

5. The method of making a casting, which 35 comprises filling a mold with molten metal, and then introducing into the interior of the molten metal material in a molten state adapted to diffuse into said molten metal and change the internal structure of the 40 casting, substantially as described.

6. The method of making a casting, which 45 comprises filling a mold with molten metal, allowing the superficial portion of the metal to cool and solidify to form a shell, and then introducing into the interior of the molten metal material in a molten state adapted to diffuse into said molten metal and change the internal structure of the 50 casting, substantially as described.

7. The method of making a casting, which 55 comprises filling a mold with quick freezing

molten material, and causing the diffusion into the interior of the molten mass of material adapted to give the casting a solid gray interior, substantially as described.

8. The method of making a casting, which 60 comprises inserting a tube into a mold so that its lower end is closed by a wall of the mold, filling said mold with molten metal, then filling said tube with molten material 65 having different characteristics from said molten metal, and then withdrawing said tube from the mold, substantially as described.

9. The method of making a one piece 65 casting having inner and outer portions of different analyses, comprising pouring molten metal about a core in a mold and during the hardening of the metal from the exterior toward the cored portion of the 70 casting causing the diffusion into the mass of molten metal which surrounded the core of material to change the analysis of the interior of the casting, substantially as described.

10. The method of making a one piece casting having inner and outer portions of different analyses, comprising pouring molten metal about a hollow core and after 75 the surface of the metal contacting with the mold has hardened, pouring molten metal of a different analysis into the interior of the core, and then withdrawing the core to permit the admixture of the two molten metals, substantially as described.

11. The method of casting a one piece roll having a chilled surface, comprising 80 making up a mold for the roll to be cast with a hollow core extending through the axis of the roll cavity in the mold, pouring 85 metal into the cavity about the core and pouring metal of different composition into the interior of the core, and then withdrawing the core to permit the molten metal in the core to mix with that on the exterior of 90 the core after the outer surface of the roll has been chilled and solidified to the desired depth, substantially as described.

In testimony whereof I have hereunto set my hand.

NED M. AUSTIN.